

## 1

3,000,821

**GREASE COMPOSITION CONTAINING LITHIUM SALT OF AN ESTER OF AN ACID PHOSPHATE**  
 Francesco Giovanni Bonmartini, Elizabeth, N.J., and Warren C. Paffenden, Mooretown, Ontario, Canada, assignors to Esso Research and Engineering Company, a corporation of Delaware  
 No Drawing. Filed June 24, 1959, Ser. No. 822,436  
 6 Claims. (Cl. 252—32.5)

This invention relates to lubricating oil compositions containing metal salts or organic substituted phosphoric acid. Particularly, the invention relates to solid grease compositions formed by thickening lubricating oils with alkali metal salts of esters of phosphoric acid.

This application is a continuation-in-part of our prior application, Serial No. 644,710, filed March 8, 1957 and now abandoned.

The phosphorus containing salts of the invention are prepared from alkali metals such as lithium and sodium. These salts impart fire retardency to the lubricant because of their high phosphorus content. In addition, they can form high dropping point greases, even in the case of lithium. Thus, while lithium salts and soaps have found widespread use as grease thickeners because of their excellent water insolubility, their application has been somewhat limited because of inability to form suitable high dropping point greases. This disadvantage is overcome by the present invention. On the other hand, salts of the alkaline earth metals, e.g. calcium, do not have the thickening effect of the corresponding alkali metal salts and form lower dropping point greases.

The thickeners of the invention are metal salts of aliphatic hydrocarbon esters of acid phosphate having the general formula



wherein R is a hydrocarbon radical such as an alkyl or alkenyl radical, and contains about 2 to 6, preferably 3 to 5, carbon atoms; Y is an alkali metal; and X is R, hydrogen or an alkali metal. The total number of carbon atoms in the compound will be about 2 to 10, preferably 3 to 8. Examples of such salts include dilithium isopropylphosphate, dilithium n-amyl phosphate, lithium n-propyl amylphosphate, sodium amyl acid phosphate, sodium diethylenephosphate, sodium hydrogen ethylenephosphate, sodium-lithium isopropylphosphate, etc.

Because of their general oil-insolubility and the difficulty of dispersing into oil, the metal salts of the acid phosphate esters are best prepared "in situ" in the lubricating oil. This is done by reacting metal base with an acid phosphate ester directly in the lubricating oil. The commercially available acid phosphate esters are generally equilibrium mixtures of mono- and di-esters which are formed by the reaction of one mole of phosphoric anhydride with 3 to 10 moles of an alcohol. A typical such reaction using 6 moles of alcohol per mole of  $\text{P}_4\text{O}_{10}$  is shown by the following equations:



The weight percentages of the mono-ester and the di-ester in these equilibrium mixtures usually varies from about 20 to 90 wt. percent of mono-ester to about 10 to

## 2

80 wt. percent di-ester, depending, of course, upon the particular esters involved and the relative proportions of alcohol and  $\text{P}_4\text{O}_{10}$  used in the reaction. However, either the mono- or di-ester may be used alone as well as mixtures in any proportions of the mono- and di-ester.

The metal base used to form the salt may be a hydroxide, oxide, or a carbonate of an alkali metal such as lithium, potassium and sodium. The metal base may be added in the form of an aqueous solution, if desired, to the mixture of oil and acid phosphate ester; however, the use of water is not necessary to stabilize the dispersion of the thickening agent in the oil.

In general, the grease composition of the invention will have an A.S.T.M. penetration of 100 to 350 mm./10, when worked 60 strokes at 77° F. and a dropping point of about 400 to 500+° F. These greases will comprise a major proportion such as 70 to 90 wt. percent, preferably 75 to 85 wt. percent of a lubricating oil, and a grease thickening amount, such as about 10 to 30 wt. percent, preferably 15 to 25 wt. percent, of the metal salt of the acid phosphate ester. The lubricating oil may be either a mineral oil or a synthetic oil.

Synthetic lubricating oils which may be used include esters of monobasic acids (e.g.  $\text{C}_8$  Oxo alcohol ester of  $\text{C}_8$  Oxo acid); esters of dibasic acids (e.g. di-2-ethyl hexyl sebacate); esters of glycols (e.g.  $\text{C}_{13}$  Oxo acid diester of tetraethylene glycol); complex esters (e.g. the complex ester formed by reacting one mole of sebacic acid with two moles of tetraethylene glycol and two moles of 2-ethyl hexanoic acid); esters of phosphoric acid (e.g., the ester formed by contacting three moles of the mono methyl ether of ethylene glycol with one mole of phosphorus oxychloride, etc.); halocarbon oils (e.g., the polymer of chlorotrifluoroethylene containing twelve recurring units of chlorotrifluoroethylene); alkyl silicates e.g. methyl polysiloxanes, ethyl polysiloxanes, methyl-phenyl polysiloxanes, ethyl-phenyl polysiloxanes, etc.); sulfite esters (e.g. ester formed by reacting one mole of sulfur oxychloride with two moles of the methyl ether of ethylene glycol, etc.); carbonates; mercaptals; poly-glycol type synthetic oils; and other synthetic lubricating oils known to the art.

The grease will generally be prepared as follows: A portion or all of the lubricating oil is mixed with the acid phosphate ester and the mixture is heated to about 100° to 250° F. At this point, the alkali metal base is added. The mixture is then further heated to about 260° to 300° F. and maintained at this temperature for about 1/2 to 3 hours to form the thickener and to dehydrate the grease. Additional lubricating oil and additives may be added to form the final grease product. If desired, the grease may also be homogenized by passing it through a Manton-Gaulin homogenizer, or a similar type of homogenizer.

The invention will be further understood by the following illustrations which include preferred embodiments of the invention.

## EXAMPLE I

A grease consisting of 20 wt. percent of the lithium salt of n-propyl acid phosphate and 80 wt. percent oil was prepared as follows: 18.0 parts by weight of n-propyl ester of orthophosphoric acid was added to 75.6 parts by weight of mineral lubricating oil having a viscosity at 100° F. at 300 S.U.S. and a viscosity index of 70. The 65 n-propyl ester of orthophosphoric acid consisted of 3

parts by weight of the mono-n-propyl dihydrogen phosphate and 7 parts by weight of the di-n-propyl monohydrogen phosphate. The mixture of these esters and oil was then heated to a temperature of 250° F. The temperature was allowed to drop to 225° F. and then 6.4 parts by weight of lithium hydroxide in the form of an aqueous solution was added to the oil-phosphate ester mixture. The resulting mixture was then further heated to a temperature of about 300° F. and maintained at this temperature for about 1 hour. The grease was then cooled to room temperature.

#### EXAMPLES II TO IV

Several more greases containing 20 wt. percent of the lithium salt of alkyl acid phosphate and 80 wt. percent of the same oil of Example I, were prepared according to the procedure of Example I.

The characteristics and compositions of the greases of Examples I to IV are given in Table I, which follows:

*Grease A.*—For comparison purposes a grease was prepared in the manner and proportions as Example I, except that ethyl lauryl monohydrogen phosphate was used.

18 parts by weight of isopropyl acid phosphate (same phosphate mixture as used in Example II) was mixed with 73.8 parts by weight of a mineral lubricating oil having a viscosity at 100° F. of 300 S.U.S. and a V.I. of 70. This mixture was heated to a temperature of about 250° F. and 6.4 parts by weight of lithium hydroxide in an aqueous solution was then added. The mixture was further heated to a temperature of about 300° F. for about one hour. The base grease thus formed was cooled to about 200° F. and 1.8 parts by weight was then added of a surface active agent sold under the trade name of Victamine C. The mixture was cooled to room temperature and tested. Victamine C has the formula:



For comparison purposes, several greases similar to that of Example V were prepared but containing different

Table I  
GREASES PREPARED FROM LITHIUM SALTS OF ALKYL ACID PHOSPHATES

| Example  | Alkyl Radical of Acid Phosphate | Wt. Ratio of mono-ester to di-ester | Micro Penetration | Dropping Point, ° F. | A.S.T.M. Penetration at 77° F. |                       | A.S.T.M. Wheel Bearing Test |
|----------|---------------------------------|-------------------------------------|-------------------|----------------------|--------------------------------|-----------------------|-----------------------------|
|          |                                 |                                     |                   |                      | Worked 60 Strokes              | Worked 10,000 Strokes |                             |
| I        | n-propyl                        | 3/7                                 | 134               | 425                  | 340                            |                       |                             |
| II       | isopropyl                       | 2.3/7.2                             | 54                | 500+                 | 180                            | 210                   | no leakage.                 |
| III      | n-butyl                         | 3/7                                 | 115               | 480                  | 310                            |                       |                             |
| IV       | n-amyl                          | 3/7                                 | 125               | 460                  | 330                            |                       |                             |
| Grease A | ethyl, lauryl                   | 100% diester                        |                   | 300                  | 230                            |                       |                             |

As seen by the preceding table, Examples I to IV resulted in high dropping point greases, while Grease A prepared from a higher molecular weight acid phosphate (total of 14 carbon atoms per molecule) formed a grease having a much lower dropping point.

Various other additives may also be added to the grease composition of the invention, such as oxidation inhibitors, dyes, metal deactivators, corrosion inhibitors, and surface active agents.

Certain surface active agents are particularly desirable in some cases in obtaining a fine dispersion of the thickener in the grease, thereby making a more efficient use of the grease thickener. The preferred surface active agents which may be used have the general formula:



wherein R is an alkyl or substituted alkyl radical of 1 to 4 carbon atoms and R' and R'' are alkyl or substituted alkyl radicals of 8 to 20 carbon atoms. Examples of such compounds include the stearyl amine salt of the stearyl amide of ethyl orthophosphoric acid, the lauryl amine salt of the lauryl amide of n-propyl orthophosphoric acid, the lauryl amine salt of the stearyl amide of ethyl orthophosphoric acid, etc. Surface active agents of the above type have been described in U.S. Patent 2,406,423.

The above-described type of surface active agent may be used in the compositions of the invention in amounts of 0.1 to 3.0 wt. percent, e.g. 0.2 to 2.0 wt. percent, based on the total weight of the grease composition, as illustrated by the following example:

surface active agents. The effect of these surface active agents is illustrated in the following table:

Table II

| Example | Surface Active Agent incorporated in the Grease <sup>1</sup>        | A.S.T.M. Penetration at 77° F. |
|---------|---------------------------------------------------------------------|--------------------------------|
| V       | None                                                                | 190                            |
|         | 1.8 wt. percent Victamine C                                         | 159                            |
|         | 1.8 wt. percent N-dodecyl-β-alanine                                 | 180                            |
|         | 1.8 wt. percent Lithium salt of lauryl alkyl phosphate <sup>2</sup> | 236                            |
|         | 1.8 wt. percent Ethomeen 18/5 <sup>3</sup>                          | 232                            |
|         | 1.8 wt. percent Stearic Acid                                        | 216                            |

<sup>1</sup> Mineral oil grease thickened with the lithium salt of isopropyl acid phosphate.

<sup>2</sup> The lithium salt of lauryl alkyl phosphate had the formula:



<sup>3</sup> Ethomeen 18/5 is an ethylene oxide condensation product containing alkyl amines.

As seen from Example V of the above table, the addition of 1.8 wt. percent of the Victamine C of the invention resulted in decreasing the A.S.T.M. penetration of the base grease from 190 to 159. This illustrates the fact that a better structure was obtained, thereby resulting in a more efficient use of the thickener. The N-dodecyl-β-alanine had a slight effect in obtaining better structure, while the other surface active agents shown in the table had a negative effect on the structure.

#### EXAMPLES VI to X

The effect of varying the concentration of the thickener in the oil was also investigated in these examples

which were prepared in a manner similar to the procedure of Example V.

*Grease B.*—For comparison purposes, a calcium grease was prepared in a manner similar to Example V, except that calcium hydroxide was used in place of the lithium hydroxide.

The formulation of the above greases in weight percent and their characteristics are summarized in Table III.

Table III

| Components                                                               | Example          |      |      |      |          |
|--------------------------------------------------------------------------|------------------|------|------|------|----------|
|                                                                          | VI               | VII  | VIII | IX   | Grease B |
| Isopropyl acid phosphate (same as in Example II) percent                 | 18.0             | 15.2 | 13.9 | 9.5  | 19.0     |
| Lithium hydroxide do                                                     | 6.4              | 5.3  | 4.4  | 3.4  | 3.8      |
| Lime—Ca(OH) <sub>2</sub> do                                              |                  |      |      |      |          |
| Vitamine C <sup>1</sup> do                                               | 1.8              | 3.0  | 2.8  | 1.9  | —        |
| Mineral lubricating oil (300 S.U.S. vis. at 100° F., V.I. of 70) percent | 73.8             | —    | —    | 77.2 | —        |
| Mineral lubricating oil (150 S.U.S. vis. at 100° F., V.I. of 90) percent | —                | 76.5 | 78.9 | 85.2 | —        |
| A.S.T.M. Penetration at 77° F. (worked 60 strokes)                       | 159              | 202  | 238  | 350  | 350      |
| Dropping Point, °F.                                                      | ( <sup>2</sup> ) | Pass | Pass | Pass | 344      |
| Boiling Water Test                                                       | —                | —    | —    | —    | —        |



<sup>2</sup> Decomposed at 425° F.

As seen by the preceding table, a much larger quantity of thickener was required in the case of the calcium grease (Grease B) and even this resulted in a relatively soft grease. On the other hand, about half as much thickener was required to obtain the same worked penetration in the corresponding lithium grease (Example IX).

What is claimed is:

1. A lubricating grease composition having an ASTM penetration of 100 to 350 mm./10 when worked 60 strokes at 77° F. and having a dropping point of about 400° F. to 500+° F. comprising a major proportion of a lubricating oil and about 10 to 30 wt. percent of a lithium salt of an ester of an acid phosphate which contains a total of 2 to 10 carbon atoms having the formula



wherein R is a C<sub>2</sub> to C<sub>6</sub> aliphatic hydrocarbon radical, Y is lithium, and X is selected from the group consisting of R, hydrogen and lithium.

2. A lubricating grease composition according to claim 1, wherein said ester of an acid phosphate is a mixture of mono- and di-esters.

3. A lubricating grease composition according to claim 1, wherein said lubricating oil is a mineral oil.

4. A lubricating grease composition according to claim 1, wherein said composition also contains 0.1 to 3.0 wt. percent of a surface active agent of the formula:



10 wherein R is an alkyl radical of 1 to 4 carbon atoms and R' and R'' are alkyl radicals of 8 to 20 carbon atoms.

5. A method of lubricating metal bearings which comprises maintaining on said bearings a lubricating grease composition having an ASTM penetration of 100 to 350 mm./10 when worked 60 strokes at 77° F. and having a dropping point of about 400° F. to 500+° F. comprising a major proportion of a lubricating oil and about 10 to 30 wt. percent of an alkali metal salt of an ester of an acid phosphate which contains a total of 2 to 10 carbon atoms having the formula



25 wherein R is a C<sub>2</sub> to C<sub>6</sub> aliphatic hydrocarbon radical, Y is lithium, and X is selected from the group consisting of R, hydrogen and lithium.

6. A process of preparing a lubricating grease having an ASTM penetration of 100 to 350 mm./10 when worked 60 strokes at 77° F. and a dropping point of about 400° F. to 500+° F. consisting essentially of a mineral lubricating oil and about 10 to 30 wt. percent of lithium salt of an ester of an acid phosphate having the formula:



35 wherein R is a C<sub>2</sub> to C<sub>6</sub> aliphatic hydrocarbon radical, Y is lithium and X is selected from the group consisting of R, hydrogen, and lithium, wherein the total number of carbon atoms in the compound is about 2 to 10, said method comprising dispersing in at least a portion of

40 said lubricating oil acid phosphate ester, heating the mixture to about 100° to 250° F., adding lithium hydroxide sufficient to form the salt and further heating at a temperature of 260° to 300° F. for a time sufficient to dehydrate the grease.

#### References Cited in the file of this patent

#### UNITED STATES PATENTS

- |           |                   |               |
|-----------|-------------------|---------------|
| 2,167,867 | Benning           | Aug. 1, 1939  |
| 2,224,695 | Prutton           | Dec. 10, 1940 |
| 2,228,659 | Farrington et al. | Jan. 14, 1941 |
| 2,274,302 | Mulit             | Feb. 24, 1942 |
| 2,406,423 | Woodstock         | Aug. 27, 1946 |